

July 5, 1932.

P. KLEM

1,865,768

METHOD OF TREATING MECHANICAL WOOD PULP

Filed Nov. 30, 1929



Inventor:  
P. Klem

By  
Renne Davis Marvin + Edmund  
attorneys

## UNITED STATES PATENT OFFICE

PER KLEM, OF OSLO, NORWAY

## METHOD OF TREATING MECHANICAL WOOD PULP

Application filed November 30, 1929, Serial No. 410,665, and in Norway November 30, 1928.

This invention relates to the manufacture of wood pulp and wood pulp products and has for its object a method of treating mechanical wood pulp, whereby the usefulness of the pulp as a constituent of paper as well as for other purposes is increased.

The invention is applicable to wood pulp of any kind, whether it has been subjected or not to a chemical treatment.

10 An important feature of the method according to the invention consists therein that the pulp is subjected to a treatment, by which that part of the pulp which is composed of fibres, fibrillae and fibre bundles is given altered properties, comprising an increased 15 flexibility and improved power of felting.

The effect aimed at may be brought about by mechanical working or by the influence of 20 chemicals or by mechanical as well as chemical means.

The result aimed at can for example be attained by separating the pulp, subsequent to 25 its having been subjected to the usual handling in suitable apparatus, into two portions according to the size of particles, whereupon one or both (or all) of said portions are each 30 separately subjected to a special treatment, after which the portions may again be united or used separately. This special treatment 35 may with respect to the coarser particles, for example, consist in a mechanical working resulting in opening (loosening) and softening 40 the fibres and making same pliable or flexible.

45 This special treatment may also be applied to the fibres at an earlier stage in the operations of producing the pulp, for example previous to the usual screening before or after separation of the so-called mill pulp or chips.

Instead of mixing the separately treated fibre grades and flour, each of the products 50 may also be further independently and separately worked, to be made applicable for different uses.

Whether the groups of fibres are mixed with one another entirely or in part or not at all, they may also be mixed with other substances of any kind before they are brought 55 into the final condition for sale or use.

In the accompanying drawing,

Fig. 1 illustrates diagrammatically an embodiment of the treatment according to the invention.

Fig. 2 illustrates a modified arrangement. 55

In the example illustrated in Fig. 1, A is the grindstone, B is a coarse screening apparatus ("bull screen" or "knotter") from which the coarser particles (slivers, splinters, knots) leave at 1, while the rest passes through 2 into the ordinary sorting system C. The sorted wood pulp thereupon passes through a system of sorting devices at D, wherein the pulp is separated into the desired number of groups, each containing the desired percentages of the 60 various particles. (This may be designated as the screening system for flour and fibre.)

The various grades or groups of pulp leave this system at 3, 4, 8 and 5. The separated groups are at E subjected to further treatment and leave at 6 to be further worked or mixed with other substances or with other groups of pulp. Other substances, such as cellulose (chemical pulp) or china clay from 65 G may be introduced into any of the grades of 70 pulp through 9.

In Fig. 2, A is the grindstone, B the coarse screening device, and K is a sorting apparatus (screen) receiving screened pulp from B. The finer particles (flour) leave this screen 80 through 16, while the coarser particles (fibres and chips) are passed into a further screen L, in which the chips are separated from the rest (which are in themselves comparatively 85 coarse particles). The chips are through 15 passed to a "refiner" to be further disintegrated. The coarser particles pass through 14 and 17 into a sorting screen M. The fine particles from M leave through 18 and unite 90 with the finer particles from 16. The coarser particles from M pass into a further screen N, wherein the remainder of chips is separated off at 19. The finer particles pass through a thickener O and into a grinding apparatus (such as a Jordan mill or beater). 95

The product is mixed with the pulp from 16 and 18. Other substances, such as cellulose in a ground or coarse condition may be introduced at 21. The resulting mixed pulp may be con- 100

veyed into thickeners at 22 or subjected to other desirable treatment.

Claim:—

6 The process of treating wood to make paper-pulp, comprising grinding the wood, separating the knots, splinters and slivers from the chips, fiber and flour produced by the grinding, screening these latter constituents to separate the flour from the fiber and 10 chips, screening the fiber and chips to separate the chips from the fiber, screening this latter fiber to separate therefrom the finer constituents, uniting the flour from the first screening with the said finer constituents, 15 passing the residue from the second screening to another screening operation, separating the chips from said residue, passing the resultant finer particles through a thickening operation, passing the product thence through a 20 beating operation to loosen and open the fiber bundles and render same pliable, mixing the pliable fibers with the products of the first and second screenings and mixing cellulose with this last mixture.

25 In testimony whereof I have signed my name unto this specification.

PER KLEM.

30

35

40

45

50

55

60